

Jan. 29, 1957

A. J. MORWAY ET AL

2,779,736

PRODUCTION OF LUBRICATING GREASES FROM OXO ESTERS

Filed Oct. 25, 1952



Arnold J. Morway  
Frederick Knobell Jr.  
Jeffrey H. Bartlett  
By L. F. Many Inventors  
Attorneys

1

2,779,736

PRODUCTION OF LUBRICATING GREASES  
FROM OXO ESTERS

Arnold J. Morway, Rahway, Frederick Knoth, Jr., Sayreville, and Jeffrey H. Bartlett, Westfield, N. J., assignors to Esso Research and Engineering Company, a corporation of Delaware

Application October 25, 1952, Serial No. 316,922

7 Claims. (Cl. 252—35)

The present invention relates to a new method of making lubricating greases and to greases produced by this method. More particularly, the invention pertains to an improved grease-making process for the production of new and improved lubricating greases of high dropping point and soft consistency over a wide temperature range.

In brief compass, the invention provides for subjecting a mixture of a high molecular weight olefin with a low molecular weight alcohol to the Oxo-ester synthesis, that is a catalytic carbonylation reaction with carbon monoxide under pressure to form directly an ester of the low molecular weight alcohol with the acid carbonylation product of the olefin charged; forming a grease-making soap from the acid radical of this ester and incorporating the soap formed into a lubricating oil to convert the latter into grease. It is desirable to combine this soap with a suitable metal salt of a low molecular weight aliphatic acid.

Prior to the present invention, soap-thickened greases of desirable hardness characteristics and high dropping points, i. e. greases melting above about 400° F. and having a smooth soft consistency over a wide temperature range have been known. These greases have been prepared by the saponification of rapeseed oil with an excess of alkali in a lubricating oil at temperatures of about 480°—500° F.

The desirable combination of excellent qualities of these greases was believed to be due largely to the use of glycerides of C<sub>22</sub> long-chain acids, such as erucic acid, as the source of the soap. Rapeseed oil and the brassidic family are the only known commercial sources for these materials. Rapeseed oil as well as all other naturally occurring ester-type fats and oils suitable for grease-making purposes have numerous other commercial uses. This situation is conducive to shortages forcing undesirable variations in grease-making procedures and grease characteristics. The present invention eliminates this difficulty.

It is, therefore, an important object of the present invention to provide soap-thickened, good-quality, high-temperature greases based on raw materials other than naturally occurring ester-type fats and oils. Another object of the invention is to provide an improved process for the production of such greases. Other objects and advantages will appear from the following description of the invention, read with reference to the accompanying drawing, the single figure of which is a schematic flow plan illustrating the invention.

It has now been found that high-temperature greases of excellent quality may be prepared by incorporating into lubricating oils, grease-thickening metal soaps obtained by the saponification of certain synthetic Oxo-esters formed by reacting mixtures of high molecular weight olefins and low molecular weight aliphatic alcohols with CO under pressure in the presence of a cobalt catalyst. The olefins should be non-aromatic and contain at least 10, say 10—20, carbon atoms per molecule, such as tetrapropylene, pentapropylene, tetrabutylene, and other polymeric olefins. Olefins produced from crack-

2

ing operations may also be used, such as cracked petroleum containing olefins in the range of C<sub>10</sub> to C<sub>20</sub>, but those having an average of about 16 carbon atoms per molecule are preferred. Suitable alcohols include the low molecular weight aliphatic alcohols having 1—3 carbon atoms, such as methanol, ethanol, etc., methanol being preferred.

It has been found highly desirable to combine the grease-making soaps of high molecular weight acids obtained from Oxo-esters with suitable metal salts of low molecular weight aliphatic carboxylic acids to form soap-salt complexes of excellent high temperature qualities. These low molecular weight acids may be used in a ratio of about 1—3 mols per mol of ester. They may have 1—5 carbon atoms per molecule, such as formic, acetic, propionic, butyric, valeric, furoic, acrylic acids, etc. The preferred low molecular weight acids are formic and acetic acids.

Metal bases suitable for the formation of simple or complex grease-thickening soaps according to the present invention include the hydroxides of alkali, alkaline earth and certain other metals, such as lithium, sodium, potassium, calcium, barium and aluminum. Alkali metal hydroxides, particularly lithium and sodium hydroxides, form complex soaps of greatest stability, highest dropping point, good water resistance and excellent susceptibility to oxidation inhibition. The total soap content of the grease may be about 6—40 wt. percent. In addition to the simple and complex soaps of the invention, conventional grease-making soaps of high molecular weight fatty acids having 10 to 30 carbon atoms, such as those derived from naturally occurring fatty materials, or suitable known grease-making salt-soap complexes may be present in proportions of up to about 50 wt. percent of the total soap content in the greases of the invention to improve high temperature or other characteristics.

Regarding suitable lubricating oil bases for greases containing the thickeners of the invention, mineral and/or synthetic lubricating oils of all types may be used, depending on the specific grease-making method employed. When the grease-making soap is formed by saponification of the Oxo-ester in the lubricating oil *in situ*, the lubricating oil used in this stage should be non-saponifiable at the conditions involved. Mineral oils, hydrocarbon polymers and some synthetic-type lubricants which resist saponification or hydrolysis, such as high molecular weight formals, ethers, etc., are suitable for this purpose. Whenever the grease-making soap is preformed and, as such, added to the lubricating oil, all types of conventional grease dispersants may be used. Lubricating oils having good volatility characteristics are also desirable, viscosities between 60 and 200 S. S. U. at 210° F., and a viscosity index suitable (generally not over 60) for soap dispersing and crystallization are preferred. However, the viscosity index of the oil may be enhanced by later blending in a higher V. I. oil during the grease manufacturing process.

The grease-making process of the invention will now be described with reference to the drawing. The process comprises two principal stages. In the first stage, i. e. the carbonylation stage designated by the reference numeral 1, Oxo-esters are prepared by subjecting mixtures of suitable olefins with low molecular alcohols of the type specified above to a catalytic carbonylation reaction with CO. The reaction may be illustrated by the equation



wherein R is an alkyl group having 1—3 carbon atoms and n is an integer of at least 10. Suitable reaction conditions in carbonylation stage 1 include temperatures of 250°—500° F., preferably about 250°—400° F., pressures of about 50—3000 atmospheres, preferably about 100—300,

and olefin to alcohol mol ratios of about 1-20, preferably about 5-15. The catalyst may be any conventional carbonylation catalyst. Cobalt present either in the free metallic state or as a suitable compound, such as the carbonyl, organic salt, soap, etc., is preferred. Inert diluents, such as cyclo-hexane, xylene, benzene, saturated hydrocarbons, etc., may be employed. When soluble catalysts are used, the ester formed is washed free of catalyst, preferably with a low molecular weight organic acid.

The product may be distilled to remove unreacted feed materials which may be recycled to the carbonylation stage. If desired, the pure acid may be recovered by hydrolysis of the ester followed by acidification, and the pure acid may then be saponified to make the grease thickener. However, it is preferred to subject the crude ester to the second stage of the process, i. e. the saponification and grease-making stage indicated at 2 on the drawing and to recover unreacted olefin and alcohol therefrom for recycling to the carbonylation stage 1 as will appear hereinafter.

The saponification stage 2 is preferably carried out in a suitable lubricating oil in situ. For this purpose, the crude or purified Oxo-ester produced in the first stage is mixed with the lubricating oil and heated therein to about 130°-170° F. Thereafter, the saponifying agent, i. e. a metal base, such as alkali hydroxide, preferably in 30-50% aqueous solution is added and the temperature raised to about 280°-325° F. When hydrolysis and saponification of the ester are complete, which is usually the case after about 1-4 hours, the temperature is raised to about 480°-520° F. maximum temperature. The grease may then be cooled to about 250° F. while stirring. At this point, other additives, such as oxidation inhibitors, etc., may be added, whereupon the grease may be further cooled while stirring to about 180°-200° F. and then poured in pans for cooling to room temperature.

When it is desired to use soap-salt complexes rather than simple soaps as the thickener of the invention, a low molecular weight carboxylic acid of the type specified may be added to the lubricating oil together with the ester or after the first heating but prior to the addition of the metal base, preferably in equi-molecular proportions with respect to the ester. Also, any additional high molecular weight acids, such as stearic acid, hydrogenated fish oil acids, etc., may be added in this case. The amount of metal base used should be sufficient completely to neutralize the acids present after hydrolysis, and preferably to leave a slight alkalinity of about 0.3-1.0% in the grease.

In the course of this saponification and grease-making stage proper, temperatures are employed at which all low molecular weight alcohol freed by the saponification reaction and introduced as impurity of the crude Oxo-ester is evaporated together with the reaction water. The same is true for any unconverted olefin introduced into the saponification mixture together with the crude Oxo-ester. In accordance with a particularly advantageous embodiment of the invention, this alcohol and unconverted olefin are passed as shown in the drawing from stage 2 to a condensation, separation and fractionation stage 3. Unconverted olefin is then recycled from stage 3 to stage 1 as indicated. Liberated alcohol may also be recovered and recycled to carbonylation stage 1, so that no fresh alcohol is required except as needed to make up for unavoidable losses. When so operating, the original olefin charge may be ultimately converted almost completely from olefin to grease in batch operation or in a fully continuous manner. This compares with a maximum olefin conversion of only about 40-50% in a single pass operation of the carbonylation stage. If desired, the grease may be passed from grease-making stage 2 to a homogenizer 4 where it may be subjected in a Gaulin or Morehouse mill type device to homogenization at high rates of shear to stabilize the grease at a desired penetration level.

Other conventional grease additives, such as antioxidants, particularly amino compounds, extreme pressure agents containing sulfur, halogen and/or phosphorus, etc., may be added to the grease in any conventional manner.

The invention will be further illustrated by the following specific examples.

*Example 1*

A 3 liter bomb equipped for heating, shaking and gas pressuring was charged with:

775 g. C<sub>13</sub> cracked petrolatum  
635 g. methyl alcohol  
9.2 g. cobalt as cobalt oleate in heptane

The bomb was then closed and pressured to 2500 lbs. with CO at room temperature. It was then heated to 302° F. where it was maintained for 21 hours. After the first hour of reaction the pressure had dropped to 1400 lbs. and the bomb was repressured with CO to 3500 lbs.

The product from the above reaction was washed with 10% acetic acid and then with water so as to remove the cobalt. It was then dried with Na<sub>2</sub>SO<sub>4</sub>, filtered and evaporated leaving 907 g. of crude ester having an ester number of 0.104 centi-equivalent per gram.

The crude methyl ester described above was saponified with alcoholic KOH in order to free a purified acid. The ester could have been used as such. However, the acid was isolated to determine its specific character.

After saponification the potassium soap was diluted with water and then extracted with naphtha to remove any inert materials, such as hydrocarbons. The aqueous layer was then acidified to liberate the acids which were then vacuum distilled. A heart cut of acid was collected for grease manufacture. This cut had a boiling point of 284°-320° F. @ 0.7 mm. Hg.

The alkali soap from the saponification may also be used directly in the manufacture of grease.

The grease was prepared as follows:

| 40 | Ingredients:                                                                  | Weight percent |
|----|-------------------------------------------------------------------------------|----------------|
|    | Hydrofol Acids 54 <sup>1</sup>                                                | 10.00          |
|    | Cracked petrolatum Oxo acid (C <sub>14</sub> )                                | 10.00          |
|    | Acetic acid                                                                   | 4.00           |
|    | Sodium hydroxide                                                              | 6.50           |
| 45 | Phenyl alpha-naphthylamine                                                    | 1.00           |
|    | Blend of naphthenic mineral oils having a viscosity of 50 S. S. U. at 210° F. | 68.50          |

<sup>1</sup> Hydrogenated fish oil acids corresponding to stearic acid in degree of saturation.

The Hydrofol Acids 54, cracked petrolatum Oxo acid and 1/2 the mineral oil were charged to a grease kettle and warmed to 150° F. The acetic acid was then added followed immediately by a 40% aqueous solution of sodium hydroxide. The temperature was raised to 300° F. After dehydration of the soap (i. e. after about 2 hours), the balance of the mineral oil was added and the temperature was raised to 500° F. Heating was then discontinued while agitating and the grease cooled to 250° F. The phenyl alpha-naphthylamine (oxidation inhibitor) was added and the grease further cooled while stirring to 200°-180° F.

Properties:

Appearance

Uniform, smooth, hard grease.

Free alkalinity as NaOH

0.32.

Penetration, 77° F., mm./10:

Unworked

180.

Worked, 60 strokes

200.

Worked, 100,000 strokes<sup>1</sup>

250.

Dropping point, ° F.

490.

Water washing, percent loss

5.

Norma-Hoffman oxidation, hours

169.

to 5 p. s. i. drop in O<sub>2</sub> pressure.

<sup>1</sup> 270 hole worker plate 1/16" diameter holes.

## Example II

The grease described in Example I was diluted with 100% of a high viscosity index lubricating oil having 375 S. S. U. viscosity at 100° F. and a viscosity index of 105. This oil addition may be made after the base grease has cooled or during the cooling cycle after complete crystallization and transition of the soap below about 300° F. The grease was then homogenized to ultimate hardness by passing through a Gaulin homogenizer at 5000 p. s. i. pressure.

## Properties:

Appearance ..... Excellent smooth yellow grease.

Penetrations, 77° F., mm./10:

|                               |      |
|-------------------------------|------|
| Unworked                      | 290. |
| Worked, 60 strokes            | 300. |
| Worked, 67,000 strokes        | 375. |
| Worked, grease rehomogenized. | 300. |

Dropping point, ° F. ..... 425.  
Copper corrosion (3 hrs. @ 210° F.).

Water washing test, percent loss. 25.

Norma-Hoffman oxidation, hours 185.  
to 5 p. s. i. drop in O<sub>2</sub> pressure.

## Example III

A 3 liter bomb equipped for heating, shaking and gas pressuring was charged with:

462 g. C<sub>13</sub> cracked petrolatum

1420 g. methyl alcohol

2.8 g. cobalt as cobalt acetate

The bomb was closed and pressured to 3800 lbs. with CO at 302° F. It was held at 302° F. for 18 hours when the final pressure had dropped to 1100 lbs.

The product from the above reaction was washed with 10% acetic acid and then with water to remove the cobalt. It was then dried with K<sub>2</sub>CO<sub>3</sub>, filtered and evaporated on the steam bath leaving 480 g. of crude methyl ester of C<sub>14</sub> Oxo acid. Its ester number was 0.163 centi-equivalents per gram, equivalent to an ester content of 38%, the remainder being unreacted olefin.

This crude methyl ester of C<sub>14</sub> Oxo acid was used as such in the manufacture of grease, in the proportions indicated below.

| Ingredients                                                                                  | Wt. Percent | Wt. Percent on an Olefin-free, Alcohol-free Basis |
|----------------------------------------------------------------------------------------------|-------------|---------------------------------------------------|
| Crude C <sub>14</sub> Methyl Ester From Cracked petrolatum (38% Ester, 62% Unreacted Olefin) | 23.60       |                                                   |
| Acid From Above Ester                                                                        | 10.00       |                                                   |
| Hydrofol Acids 54.                                                                           | 8.50        | 10.00                                             |
| Acetic Acid (Glacial)                                                                        | 3.40        | 4.00                                              |
| Sodium Hydroxide                                                                             | 5.50        | 6.50                                              |
| Phenyl alpha-Naphthylamine                                                                   | 0.85        | 1.00                                              |
| Blend of Naphthenic Mineral Oils Having a Viscosity of 50 S. S. U. at 210° F.                | 58.15       | 68.50                                             |

The crude ester, Hydrofol Acids and 1/2 of the mineral oil were charged to a kettle and warmed to 150° F. Then the acetic acid was charged, followed immediately by a 40% aqueous solution of the sodium hydroxide. Heating was continued to 300° F. where the balance of the mineral oil was added. During this heating period before the addition of the balance of the mineral oil, water and alcohol were vaporized along with olefins that were present in the crude ester. The product was further cooled to 200° F.

|             |                                                                    |      |                                            |  |
|-------------|--------------------------------------------------------------------|------|--------------------------------------------|--|
| Properties: | Appearance.....                                                    |      | Excellent Smooth, Hard, Homogeneous Grease |  |
|             | Percent Free Alkalinity as NaOH.....                               | 0.27 |                                            |  |
|             | Penetration, 77° F., mm./10:                                       |      |                                            |  |
| 5           | Unhomogenized                                                      | 130  | 167                                        |  |
|             | Worked, 60 Strokes                                                 | 246  | 240                                        |  |
| 10          | Worked, 60,000 Strokes                                             |      | 310                                        |  |
| 15          | Dropping Point, ° F.....                                           | 450+ |                                            |  |
|             | Percent Loss in Water Washing Test.....                            | None |                                            |  |
| 20          | Norma-Hoffman Oxidation, Hours to 5 p. s. i. Drop in Pressure..... | 137  |                                            |  |

The present invention is not limited to the specific figures of the foregoing examples. The relative proportions of the materials used may be varied within the limits indicated in the specification to obtain products of varying characteristics.

## What is claimed is:

1. A process for making grease which comprises contacting in a carbonylation stage a non-aromatic olefin having about 10 to 20 carbon atoms with an aliphatic alcohol having about 1 to 3 carbon atoms and carbon monoxide in the presence of a carbonylation catalyst at conditions conducive to the formation of an ester of said alcohol with an acid having 1 carbon atom more than said olefin, recovering a mixture of said ester with unconverted olefin, introducing said mixture into a mineral lubricating oil, subjecting the resulting mixture to saponification with a metal base at a grease-making temperature of about 280° to 325° F. to form a grease while driving off unconverted olefin and alcohol freed by said saponification reaction, cooling the grease and returning said unconverted olefin so driven off to said carbonylation stage, said lubricating oil being non-saponifiable at the conditions of said saponification.

2. The process of claim 1 wherein said alcohol so driven off is returned to said carbonylation stage.

3. The process of claim 1 wherein said grease is heated to a temperature of about 480° to 520° F. subsequent to said saponification.

4. The process of claim 3 in which a high molecular weight fatty acid having from about 10 to 30 carbon atoms derived from naturally occurring fatty material and a low molecular weight carboxylic acid having from about 1 to 5 carbon atoms per molecule is introduced into said lubricating oil with the mixture of said ester and unconverted olefin.

5. The process of claim 4 wherein said high molecular weight fatty acid is hydrogenated fish oil acid and said low molecular weight carboxylic acid is acetic acid.

6. The process of claim 1 wherein said metal is selected from the group consisting of alkali metals, alkaline earth metals and aluminum.

7. The process of claim 6 wherein said metal is sodium.

## References Cited in the file of this patent

## UNITED STATES PATENTS

|           |                 |                |
|-----------|-----------------|----------------|
| 2,271,619 | Bradshaw et al. | Feb. 3, 1942   |
| 2,449,312 | Murray et al.   | Sept. 14, 1948 |
| 2,468,099 | Morway          | Apr. 26, 1949  |
| 2,470,859 | Pavlic          | May 24, 1949   |
| 2,575,286 | Morway et al.   | Nov. 13, 1951  |
| 2,576,032 | Morway et al.   | Nov. 20, 1951  |
| 2,542,767 | Gresham et al.  | Feb. 20, 1951  |
| 2,594,341 | Owen et al.     | Apr. 29, 1952  |
| 2,606,153 | Holdstock       | Aug. 5, 1952   |
| 2,607,787 | Mason           | Aug. 19, 1952  |
| 2,628,195 | Allison et al.  | Feb. 10, 1953  |
| 2,628,938 | Whitney         | Feb. 17, 1953  |
| 2,648,694 | Mason           | Aug. 11, 1953  |